

E. M. CHADBOURNE,  
ASPHALT ROADWAY.  
APPLICATION FILED MAY 29, 1911.

1,098,710.

Patented June 2, 1914.



Witnesses

Thomas Durant  
Robert S. Brown.

Inventor  
Edward M. Chadbourne

By *Charles V. Church*  
his Attorney

# UNITED STATES PATENT OFFICE.

EDWARD M. CHADBOURNE, OF SAN FRANCISCO, CALIFORNIA.

## ASPHALT ROADWAY.

1,098,710.

Specification of Letters Patent.

Patented June 2, 1914.

Application filed May 29, 1911. Serial No. 630,066.

To all whom it may concern:

Be it known that I, EDWARD M. CHADBOURNE, a citizen of the United States, residing at San Francisco, in the county of 5 San Francisco and State of California, have invented a certain new and useful Improvement 10 in Asphalt Roadways; and I do hereby declare the following to be a full, clear, and exact description of the same, reference being had to the accompanying drawings, forming a part of this specification, and to the figures and letters of reference marked thereon.

This invention relates to the construction 15 of pavement for roadways and more especially to that type wherein the surface is formed by a rock or stone aggregate combined with an asphaltic binder which is substantially non-fluid at ordinary temperatures, but capable of being rendered limpid or liquid by heat. The surface layer is usually supported by a suitable foundation, such as cement concrete; macadam; approved practice indicating the desirability 20 of forming the surface of the base with pockets or irregularities as set forth, for instance, in my prior Patents Nos. 956,940, 965,562 and 982,247 and the present invention will be described under the assumption that a 25 foundation of the character stated, is employed. In so far as the pavement produced is concerned, it is the object of the invention to form a surface layer which will be a homogeneous mass, substantially free from 30 voids and with such proportions of aggregate and binder as will afford a maximum resistance to wear and displacement under traffic conditions and at the same time conform to approved practice with respect to 35 surface conditions and resiliency for absorbing shock and vibration without disintegration.

In so far as the process of producing the pavement is concerned, the objects of the invention are, to reduce the number of steps and machinery necessary for handling and combining the ingredients; to bring the ingredients together in such manner that the voids in the aggregate are filled by capillary 45 action and downward penetration from above, and to permit of the use of a cheap and easily prepared or obtained aggregate. 50 Attempts have heretofore been made to

produce a homogeneous layer of aggregate and asphaltic binder for roadway surfaces. 55 For instance, it has been proposed to grade the aggregate and to combine the graded material in certain proportions and sizes, and to mix the binder therewith by agitation and heat, the completely mixed aggregate and binder being carried to and deposited on the roadway where it is spread and rolled, but such operations do not result in a 60 homogeneous mixture, as the particles stick together when suddenly cooling, forming 65 masses, some or all of which have larger proportions of certain sizes of the aggregate than others, and the binder is caused to drain out because of its hot liquid state, and only coat the particles and not fill the voids. 70 When laid and rolled not only is it impossible to prevent the leaving of a percentage of voids, but owing to the irregularity of the mixture, the surface layer will wear and disintegrate irregularly. It has also been 75 proposed to pour a hot asphalt binder over a layer of cold aggregate with a large percentage of voids amounting to about 50% of the total volume, but owing to the rapid cooling of the binder, when it comes in contact with the cold aggregate, irregular penetration results; furthermore, the adhesion 80 between the aggregate and the asphalt binder is not strong or lasting. A great quantity of asphalt binder is used endeavoring to fill the voids in the aggregate with the result that the asphalt binder becomes a 85 wear resistant material, a use for which it was never intended.

In accordance with the present invention 90 the foundation is prepared preferably of cement concrete, and suitable provision at the top surface such as pockets or irregularities to bond the surface to the base more securely. Upon this foundation there is 95 spread evenly a layer of hot aggregate with which the binder is to be combined. The aggregate is composed of broken natural stone mixed with sand or sand alone, the larger pieces of which are of less diameter than the thickness of the layer of which they form a part. The aggregate of sand should be such that it has from 25% to 40% voids as it is within these limits that effective capillary action and absorption will 100 draw the binder down and cause the same to

spread uniformly through the mass or layer of aggregate. Should the percentage of voids be larger, the interstices are too large to hold the hot liquid asphalt binder in suspension by surface tension or for capillarity to act effectively, with the result that the asphalt binder would flow away and be of no use, it simply coating some particles of aggregate and leaving the rest bare. Should the percentage of voids be smaller, capillary action and downward percolation are blocked, probably because the finer particles float in the binder and close the passageways or render the binder too viscous to feed by capillarity. The aggregate preferably employed consists of 50% broken stone such as will pass a  $\frac{1}{2}$ " or 1" mesh mixed dry with 50% of sand, having between 25% and 40% of voids, or a torpedo sand alone with approximately the same quantity of voids. This aggregate is heated to a high temperature and distributed in an even layer over the base and while in this hot condition a binder containing a large percentage of asphalt, said binder being substantially non-fluid in ordinary temperature, but capable of being rendered liquid or fluid by heat is poured over the surface of the same. The layer of aggregate preferably approximates in thickness the thickness of the surface layer desired and the thickness of the layer of binder is such that approximately the whole of it will be absorbed by the heated aggregate. In other words, the binder equals the void volume of the aggregate. The practical result of the action of pouring the binder on the hot aggregate is to render the former limpid and in condition to feed by capillary action and downward percolation into the aggregate. This action takes place almost immediately and although there is a large volume of binder to be absorbed in proportion to the volume of each of the finer particles of the aggregate, the stored heat due to the presence of the pieces of aggregate is sufficient to effectively keep the binder a liquid and prevent the same from solidifying as it penetrates the mass of aggregate.

The limits within which the capillary action will be effective in causing a normally non-fluid asphaltic binder to be effectively absorbed and held in suspension until solidification, it is believed are fairly well defined by the percentage of voids in the aggregate and to lie, as before stated, between 25 and 40%. To bring the percentage of voids within these limits, a comparatively rough grading is all that is necessary with any crushed rock or gravel and the addition of ordinary sand is sufficient to either reduce the percentage of voids when too great or to increase the percentage of voids when too small.

The accompanying drawing shows a sec-

tion of the roadway and illustrates the process of laying the same.

In said drawing "A" is the cement concrete base; "B" is a hot layer of aggregate having approximately 50% of large particles  $a$  and 50% of small particles  $a'$ , the latter having between 25 and 40% of voids.

"C" is a layer of normally non-fluid asphaltic binder poured on the hot aggregate.

"E" is a finished section in which the binder, has fed down by capillary attraction, and percolation into the layer of aggregate so as to completely fill the voids therein.

After the binder has been melted and absorbed and the layer is partly cooled, the surface is preferably smoothed and evened by rolling with a smooth roller.

Having thus described my invention, what I claim as new and desire to secure by Letters Patent of the United States, is:

1. The method of pavement construction which consists in providing an aggregate composed of a mixture of wear resistant stone and sand, the interstices in the sand being of such size as to exert capillary attraction and absorption, on an asphaltic binder capable of being liquefied by heat, then heating and spreading the mixture of stone and sand on a suitable foundation in a layer with its surface conforming to the desired grade and finally filling the interstices therein from the top by capillary action and percolation with a normally non-fluid asphaltic binder rendered limpid by heat, whereby a homogeneous layer is produced having no excess of either binder or aggregate.

2. The method of pavement construction which consists in spreading on a supporting foundation a layer of heated aggregate having from 25% to 40% of voids, and in applying thereto an asphalt binder capable of being rendered limpid by heat whereby the stored heat in the aggregate retains the binder in a liquid state until it can be absorbed by downward percolation and capillary attraction into the aggregate.

3. The method of pavement construction which consists in providing a layer of heated aggregate composed of a mixture of wear-resistant stone and sand with its surface substantially conforming to the desired grade and the voids of which are of such size as to absorb and retain by surface tension a liquid bituminous compound, and in distributing over said aggregate a substantially uniform layer of bituminous compound non-fluid at ordinary temperatures, but capable of being liquefied by heat, whereby the bituminous compound is absorbed and held in the voids of the aggregate until cool and non-fluid.

4. The method of pavement construction which consists first in preparing a suitable

foundation; secondly, spreading on said foundation a layer of heated aggregate having not less than 25% or more than 40% of voids; and thirdly, pouring over said 5 layer of heated aggregate a binder capable of being rendered limpid by heat but which at ordinary temperatures is non-fluid where- by the voids in the aggregate are filled from above by penetration.

EDWARD M. CHADBOURNE.

Witnesses:

M. T. MARRIAM, Jr.,  
THOS. J. STRAUB.